

## UNITED STATES PATENT OFFICE

ALBERT LEVY MOND, OF LONDON, ENGLAND, ASSIGNOR TO I. G. FARBENINDUSTRIE AKTIENGESELLSCHAFT, OF FRANKFORT-ON-THE-MAIN, GERMANY

PROCESS OF PRODUCING CASTINGS OF MAGNESIUM AND HIGH GRADE MAGNESIUM ALLOYS

No Drawing. Application filed December 14, 1929, Serial No. 414,240, and in Great Britain December 19, 1928.

This invention relates to the art of making castings of magnesium and high grade magnesium alloys.

An object of the present invention is to provide a method for producing castings of the aforesaid metals in green sand moulds—i. e. unbaked moulds still containing the moisture requisite to render the sand mouldable. Another object is to obtain castings which are—by virtue of a protective layer formed on the castings incidentally with the casting process—resistant to corrosion in a higher degree than hitherto feasible. Such protective layers are known per se, but their formation required a special treatment, i. e. a distinct operation entirely independent of the casting process. Other objects of the invention will appear from the following.

In U. S. A. Patent 1,463,609, a process of casting magnesium and magnesium alloys is described which consists in applying to the mould, prior to casting the metal, a substance which is capable of giving off, in contact with the molten metal, a gaseous substance which is more easily oxidizable than magnesium. In U. S. A. Patents 1,584,072 and 1,614,820, an improved modification of this process is described, inasmuch as the moulds are prepared from a mixture of green sand with non-metallic substance incapable of reaction with the metal and adapted, when heated by the heat emitted from the cast metal, to form on the surface of the casting a layer preventing the casting from being spoilt by the access of air and water vapour. As suitable substances of this kind are mentioned sulphur, boric acid, oxalic acid compounds, bicarbonates, urea and mixtures of these substances. It will be noted that the substances thus claimed are supposed to be incapable of reaction with the metal and it further appears that the protective layer on the metal is only present during the casting operation, generally in the form of a gas.

Inasmuch as urea, when employed in mixture with green sand, had given satisfactory results and as it is well known that urea under certain conditions is decomposed under the influence of heat into an ammonium salt, namely ammonium isocyanate, with the liber-

ation of ammonia, during casting when using moulding sand containing urea and as we have actually observed the presence of ammonia we tried other ammonium compounds for the same purposes.

It is further known that the resistance of articles made of magnesium and magnesium alloys to corrosion is, by a superficial treatment with fluoride solutions, considerably increased, probably owing to the formation of a dense, although extremely tenuous, protective layer of a magnesium-fluorine compound. With the object of forming a permanent protective layer of this kind incidentally with the casting process on the cast articles—as distinguished from the temporary protection afforded by the known substances applied in the casting processes according to the above-mentioned patents—I employed an ammonium salt which is combined with fluorine, i. e. ammonium fluoride, in mixture with green sand as a means for creating a neutral atmosphere between the sand and the molten solidifying metal. However, the hygroscopic properties of ammonium fluoride provided to be a great disadvantage, inasmuch as ammonium fluoride in contact with sand and water or moisture, readily decomposes giving off ammonia vapours. The moulds thus rapidly become impoverished with respect to the protective substance and this detrimental effect is still further promoted by the heating of the sand in the course of casting. The sand therefore practically can not be used over again without readdition of ammonium fluoride.

A further object of the present invention is therefore, to avoid the detrimental effects of such hygroscopicity in the material constituting the mould.

This object can be fulfilled in numerous different ways. It may be either achieved by embodying in the sand, together with ammonium fluoride, an acid which is capable of absorbing ammonia, or by employing, instead of ammonium fluoride, a complex chemical compound of said substance having a smaller tendency to decompose under the influence of moisture and heat.

Thus, according to one embodiment of the

invention, I employ a fluorine compound which is non-hygroscopic and which at the same time has the property, when coming into contact with the molten metal, of creating a neutral atmosphere and of providing a protective layer on the cast metal.

I have found that a suitable substance of this kind is the acid ammonium fluoride or ammonium hydrofluoride  $\text{NH}_4\text{F}$   $\text{HF}$ , which 10 when mixed with green sand in amounts preferably ranging between 3 and 5 per cent ensures perfect castings. As practically no decomposition of the salt occurs the sand may be repeatedly used without further addition 15 of this protective ingredient.

By way of example I have further found that a substance which in contact with water yields a non-hygroscopic fluoride compound by decomposition, namely ammonium silico-fluoride, when admixed to the sand in the aforementioned proportions, also gives satisfactory results.

The property of this salt of decomposing, in the presence of water, to form a non-hygroscopic fluoride offers the advantage that by its employment the free moisture of the green sand is simultaneously reduced, i. e. part of the moisture of the sand is withdrawn. This is probably due to the fact that an equilibrium is established between ammonium silico-fluoride and water, which can be explained by the following equation:



35 This property can be proved by the simple experiment of dissolving ammonium silico-fluoride in water, when after a short while silicic acid is precipitated, which is capable 40 of absorbing water. In addition free hydrofluoric acid is formed. When using ammonium silico-fluoride in practice it is advantageous, before forming the mould, to store the sand to which the silico-fluoride has been 45 admixed, preferably in a quantity amounting to about from 3 to 5 per cent, for some time, until the reaction has taken place between the ammonium silico-fluoride and the water present in the green sand and until the 50 silica gel formed has absorbed some of the moisture in the green sand.

If this precaution be omitted the sand will swell owing to the increase in volume of the silica gel and if such sand be used immediately 55 the impression of the pattern will become distorted. The free hydrofluoric acid or other fluorine compounds that may be produced during casting have the property of forming an anti-corrosive layer on the metal itself.

According to a modification of the invention, I may use a hygroscopic fluorine compound such as ammonium fluoride and associate therewith a substance adapted to obviate the detrimental effects of the hy-

groscopicity of such compound, for example by combining or absorbing or adsorbing the decomposition products.

I have found that oxalic acid, when added to a sand containing the hygroscopic ammonium fluoride, very efficiently reduces the decomposition of the latter in contact with the moisture of the sand. Thus a green sand thoroughly mixed with about 5 percent of ammonium fluoride and about 3 percent of oxalic acid shows hardly any decomposition and is suitable for casting magnesium and magnesium alloys, at the same time providing the finished castings with a protective layer of a fluoride compound. 75

I have further found that the tendency of the ammonium silico-fluoride to cause a swelling of the moist moulding sand, thus necessitating a storing of the sand before using it for moulding, is also substantially 80 checked by incorporating, in the sand, oxalic acid, preferably also in a quantity of about 3 percent, together with ammonium silico-fluoride. In this case, a storing of the sand before use is no longer necessary. 85

The substances and compositions hereinbefore described, may in the case of small castings be employed by themselves in amounts preferably not exceeding 15 percent. In the case of larger castings, however, it is frequently advisable to further add one or more of the protective substances disclosed in the specification of the U. S. A. Patents 1,463,609, 1,584,072 and 1,614,820, preferably small percentages of sulphur and/or boric acid, to the sand, so as to efficiently prevent local scorches. 90

It will be understood that the application 95 of the substances hereinbefore described is not limited to impregnating the sand by admixing these substances, although this is generally the most economical and simple way of applying them. Any mode of application which will ensure contact between the molten metal and the protective substances disclosed 100 within the mould falls within the scope of the present invention. Thus, for example, it is also sufficient to impregnate the sand constituting the inner surface of the finished mould with the substances named before casting 105 the metal into the mould. 110

I claim:

1. A process of producing castings of magnesium and high grade magnesium alloys which comprises bringing ammonium fluoride and an acid capable of absorbing ammonia into contact with the surface of the molten metal within the mould. 120

2. A process of producing castings of magnesium and high grade magnesium alloys which comprises bringing ammonium fluoride and an acid of the group consisting of hydrofluoric acid and oxalic acid into contact with the surface of the molten metal within the mould. 125

3. The method of making green sand moulds for casing a magnesium and magnesium alloys which comprises impregnating at least the inner surface of the mould with ammonium fluoride and an acid capable of absorbing ammonia.

4. The method of making green sand moulds for casting magnesium and magnesium alloys which comprises impregnating at least the inner surface of the mould with ammonium fluoride and an acid of the group consisting of hydrofluoric acid and oxalic acid.

5. A process of producing castings of magnesium and high grade magnesium alloys which comprises bringing an inert protective substance and ammonium fluoride and an acid capable of absorbing ammonia into contact with the surface of the molten metal within the mould.

6. A process of producing castings of magnesium and high grade magnesium alloys which comprises bringing sulphur and ammonium fluoride and an acid of the group consisting of hydrofluoric acid and oxalic acid into contact with the surface of the molten metal within the mould.

7. The method of making green sand moulds for casting magnesium and magnesium alloys which comprises impregnating at least the inner surface of the mould with an inert protective substance and ammonium fluoride and an acid capable of absorbing ammonia.

8. The method of making green sand moulds for casting magnesium and magnesium alloys which comprises impregnating at least the inner surface of the mould with sulphur and ammonium fluoride and an acid of the group consisting of hydrofluoric acid and oxalic acid.

In testimony whereof I have hereunto set my hand.

ALBERT LEVY MOND.

45

50

55

60

65